

## UNITED STATES PATENT OFFICE

2,098,042

## STENCIL SHEET

Shinjiro Horii, Tokyo, Japan

No Drawing. Application May 27, 1936,  
Serial No. 82,090

1 Claim. (CL. 41—38.6)

This invention relates to stencil sheets for use in duplicating manuscript or typewritten matters and the like, consisting of a sheet of fibrous material provided with a coating of an ink-resisting composition, and which can be stencilized by the pressure of a stylus, or the type of a type-writing machine.

Heretofore the stencil sheets of this kind have been made generally of a base sheet of fibrous paper coated with a coating material comprising a protein substance, such as glue or gelatine, or a cellulose compound, such as cellulose nitrate, both being in combination with some suitable softening materials. The effective softening materials are usually vegetable oils, fats and fatty acids.

According to the present invention the stencil sheets are prepared by the fibrous sheets, such as Japanese Yoshino paper, being coated with a composition including a gelatinous organic colloid, such as gelatine, in admixture with mono- or di-oleic acid ester of glycerin, an emulsifying agent, such as Turkey-red oil, and pigments.

With regard to stencil sheets of this character it may be also stated that the coating composition thereof comprises gelatine together with softening materials, such as (1) naphthenic acid esters, e. g. ethyl naphthenate, a glycol naphthenate and glyceryl naphthenate, and (2) a higher hydroxy fatty acid ester of a di-hydric alcohol such as a ricinoleic acid ester of a glycol.

The mono- or di-oleic acid ester of glycerin is an oily material which is more easily emulsifiable with gelatine solution than the natural oils or fats. It is miscible with mineral oils. It is neither sticky nor tacky and without the defect of becoming rancid on keeping. Consequently the stencil sheets produced in accordance with the present invention possess certain advantages over the sheets produced by the use of triglycerol esters of fatty acids, in that they have not the defect of becoming sticky on keeping, and are capable of being more easily and sharply stencilized by only a light pressure.

In the carrying out of the invention, a gelatine is swelled by being soaked in water, whereupon it is dissolved in hot water. The solution is then mixed and emulsified with Turkey-red oil, mono- or di-oleic acid ester of glycerine and other suitable softening agents, such as mono- or di-oleic acid ester of ethylene glycol, ethyl oleate, naphthenic acid glycerides, oleic acid, and mineral oils, in admixture with some suitable pigments, such as Prussian blue, ultramarine blue, organic lakes, kaolin, powdered talc or agalmatolite, barytes, blanc fixe. The mixture is then applied to a base sheet, such as Japanese-Yoshino paper, in the usual manner.

The proportions of the ingredients of the composition may vary according to circumstances. The following is an example:

|                           | Parts by weight |
|---------------------------|-----------------|
| Gelatine                  | 10              |
| Oleic acid mono-glyceride | 25              |
| Glycol oleate             | 10              |
| Oleic acid                | 10              |
| Heavy mineral oil         | 10              |
| Turkey-red oil            | 25              |
| Ultramarine blue          | 15              |
| Kaolin                    | 10              |
| Powdered agalmatolite     | 10              |
| Water                     | 200             |
| Hexamethylentetramine     | 1               |
| Preservative              | 1               |
|                           | 30              |

A hardening agent, such as formalin or hexamethylentetramine, and a preserving agent, such as phenols or their derivatives, may be added to the coating mixture.

What I claim is:

A stencil sheet, comprising a base of fibrous material material coated with a composition including gelatine, mono- or di-oleic acid ester of glycerine, mono- or di-oleic acid ester of ethylene glycol, oleic acid, Turkey-red oil, a heavy mineral oil, Prussian blue, organic lakes, kaolin, powdered agalmatolite, hexamethylentetramine, and a preservative.

SHINJIRO HORII.